

## UNITED STATES PATENT OFFICE

2,432,095

## LUBRICATING COMPOSITION

Delton R. Frey, East Cleveland, Ohio

No Drawing. Application December 29, 1941,  
Serial No. 424,823

13 Claims. (Cl. 252—46.7)

1

This invention relates, as indicated, to the stabilization of liquid hydrocarbon compositions. The term "liquid hydrocarbon compositions" as used herein is intended to include liquid compositions which are essentially derivatives of petroleum, naturally occurring oils of the types represented by animal, vegetable and marine oil and derivatives of the same.

More specifically this invention relates to the stabilization of liquid hydrocarbon compositions which are essentially mineral oil and particularly mineral oil of the character commonly employed as lubricants. My invention, however, is likewise applicable to the stabilization of lighter fractions of petroleum such as are used for fuels. Liquid hydrocarbon compositions of the character above identified are subject during storage, handling and particularly during use, to deterioration which may be occasioned either by oxidation or polymerization, and such deterioration usually proceeds at an accelerated rate when, for example, the liquid hydrocarbon composition is subjected to elevated temperatures and similar conditions encountered when the same are used as lubricants in internal combustion engines.

This deterioration, which, as indicated, may occur either during storage, handling or use, is generally manifested by discoloration of the liquid hydrocarbon body; generation within the body of flocculent material; the precipitation from the body of the more serious types of deterioration products such as sludge; and the deposit of varnish or shellac-like deposits on metallic surfaces with which the compositions come in contact especially during use.

Inasmuch as deterioration is usually accelerated by the severe conditions, such as temperature, to which the hydrocarbon composition is subjected, it will be observed that my invention is particularly suited for the stabilization of hydrocarbon compositions such as mineral lubricating oils used as the lubricant in the crank case of internal combustion engines whether of the ignition or Diesel type. My invention is particularly applicable to the stabilization of lubricants used in Diesel engines on account of the more severe stresses to which the lubricating composition is subjected in that type of engine.

It is a principal object of my invention therefore to provide for the stabilization of compositions of the character defined in order to reduce the tendency of the same to decomposition, particularly in the manner indicated.

It will also be observed that the addition agents employed for the described purposes, especially when prepared in the manner hereinafter more specifically defined, are in themselves new compositions of matter.

Other objects of my invention will appear as the description proceeds.

2

To the accomplishment of the foregoing and related ends, the invention, then, comprises the features hereinafter fully described, and particularly pointed out in the claims, the following description setting forth in detail certain illustrative embodiments of the invention, these being indicative, however, of but a few of the various ways in which the principle of the invention may be employed.

10 Broadly stated, this invention comprises the stabilization of liquid hydrocarbon compositions of the character previously identified, by the inclusion therein of a minor proportion of an oil-soluble compound having in the same molecule a cycloaliphatic radicle and the phosphite radicle.

15 The compounds contemplated for use by my invention are believed to have the following structure:

20



wherein X is oxygen or sulphur; P is phosphorus; 25 A is a cycloaliphatic radicle; and B and C are the same or different radicles selected from the class consisting of hydrogen, a metal and any organic radicle.

In the foregoing structure formula indicative of 30 the compounds which are useful as addition agents in the compounded lubricants of my invention it will be observed that the location of the cycloaliphatic radicle is not critical, i. e., it may be at B or C instead of at A as indicated;

35 one or more of the radicles A, B and C may be a cycloaliphatic radicle; and when for example the cycloaliphatic radicle is at A, then B and C may be the same or different radicles selected from the class consisting of hydrogen, the metals and any organic radicle. The metals which may be used 40 are those which are capable of producing oil-soluble derivatives of the remainder of the molecule. Generally the polyvalent metals are preferred and the following metals will be found particularly suitable for use, the same being arranged in the order of their preference:

|    |           |         |
|----|-----------|---------|
| 50 | Calcium   | Zinc    |
|    | Magnesium | Cadmium |
|    | Barium    | Cobalt  |
|    | Beryllium | Nickel  |
|    | Strontium | Tin     |
| 55 | Aluminum  | Silver  |
|    | Chromium  | Copper  |

As previously indicated, any organic radicle 60 may be utilized at one of the positions A, B or C (see B or C for illustration where the cycloaliphatic radicle is at A).

phatic radicle is positioned at A) and in this connection reference may be had to the following table for a classification and identification of specific organic radicles which may be utilized for this purpose.

Table II

## I. Hydrocarbon radicles

## (A) Alkyl radicles

Amyl (n, iso, sec. and tertiary)  
Lauryl  
Cetyl  
Carnaubyl  
Ceryl  
Montanyl  
Mellisyl  
Myricyl  
Lacceryl  
Ptyllicyl

## (B) Aryl radicles

Phenyl  
Xenyl  
Naphthyl (alpha- and beta-)  
Anthracetyl  
Phenanthryl

## (C) Cyclo-alkyl radicles

Cyclopentyl  
Cyclohexyl  
Cycloheptyl  
Cyclohexyl-cyclohexyl

## (D) Alkylated aryl radicles

Radicles formed by the alkylation of aryl radicles, such as those listed above (B), with any of the alkyl radicles, e. g., those listed above (A), or with any of the following:

Methyl  
Ethyl  
Propyl (n-, and iso-)  
Butyl (n-, iso- and sec-)

Specific examples of alkylated aryl radicles are as follows:

Cresyl  
Xylyl  
Trimethyl-phenyl  
Ethyl-phenyl  
Tetra-ethyl-phenyl  
t-Amyl-phenyl  
Lauryl-phenyl  
Cetyl-phenyl  
Cetyl-n-xylyl  
Methyl-naphthyl  
Iso-propyl-naphthyl  
t-Ani-l-naphthyl  
Lauryl-naphthyl  
Cetyl-naphthyl  
Iso-propyl-xenyl  
t-Ani-xenyl  
Lauryl-xenyl

## (E) Alkylated cyclo-alkyl radicles

Radicles formed by the alkylation of cyclo-alkyl radicles such as those listed above (C), with any of the alkyl radicles, such as those listed above.

Specific examples are:

Methyl-cyclohexyl

Dimethyl-cyclohexyl

t-Amyl-cyclohexyl

Lauryl-cyclohexyl

Cetyl-cyclohexyl

## (F) Cyclo-alkylated aryl radicles, e. g.,

Cyclo-ethyl-phenyl  
Cyclo-ethyl-xenyl  
Cyclo-ethyl-naphthyl

## (G) Arylated-alkyl radicles, e. g.,

Benzyl

Phenyl-ethyl

Phenyl-amyyl

Phenyl-lauryl

Phenyl-cetyl

Xenyl-n-ethyl

Xenyl-ethyl

Naphthyl-methyl

Naphthyl-ethyl

## (H) Cyclo-alkylated alkyl radicles, e. g.,

Naphthene

Hexahydro-phenyl

Cyclo-ethyl-ethyl

Cyclohexyl-ethyl

## (I) Arylated cyclo-alkyl radicles, e. g.,

Phenyl-cyclohexyl

Xenyl-cyclohexyl

Naphthyl-cyclohexyl

## (J) Mixed radicles, e. g.,

Methylcyclohexyl-phenyl

Amylcyclohexyl-phenyl

Cyclo-ethyl-cresyl

Cyclo-ethyl-xylyl

Cyclo-ethyl-amy-phenyl

Cyclo-ethyl-benzyl

Xylyl-cyclo-ethyl

Lauryl-phenyl cyclohexyl

Cetyl-phenyl cyclohexyl

Phenyl-methylcyclohexyl

Phenyl-amylcyclohexyl

Xylyl-methylcyclohexyl

Benzyl-cyclohexyl

Benzyl-methylcyclohexyl

Methylcyclohexyl-amy

Methylcyclohexyl-lauryl

## II. Oxygen-containing organic radicles

(A) Of the ether type, e. g.,  
Methoxy-phenyl  
Ethoxy-phenyl  
Lauroxy-phenyl  
Cyclohexoxy-phenyl  
Phenoxy-phenyl  
Phenoxy-naphthyl  
Phenoxy-cyclohexyl  
Phenoxy-ethyl  
Phenoxy-lauryl  
Phenoxy-cetyl  
Amyl-phenoxy-ethyl  
Phenyl-ethoxy-ethyl  
-C<sub>6</sub>H<sub>4</sub>-O-C<sub>2</sub>H<sub>4</sub>-(derived from di-ethylene glycol)

## (B) Of the ketone type, e. g.,

Acetyl-phenyl  
Acetyl-xenyl  
Acetyl-naphthyl  
Acetyl-lauryl  
Acetyl-cetyl  
Acetyl-cyclohexyl  
Acetyl-naphthene  
Lauroyl-phenyl  
Benzoyl-phenyl  
Benzoyl-naphthyl  
Benzoyl-cyclohexyl  
Benzoyl-naphthene  
Benzoyl-lauryl  
Benzoyl-cetyl  
Stearoyl-phenyl  
Stearoyl-xenyl  
Stearoyl-naphthyl  
Stearoyl-amyl  
Stearoyl-lauryl  
Stearoyl-cetyl  
Stearoyl-phenoxy-phenyl  
Stearoyl-cyclohexyl  
Stearoyl-naphthene  
Naphthenoxy-phenyl  
Naphthenoxy-xenyl  
Naphthenoxy-naphthyl  
Naphthenoxy-amyl  
Naphthenoxy-lauryl  
Naphthenoxy-octyl  
Naphthenoxy-phenoxy-phenyl  
Naphthenoxy-cyclohexyl  
Phenoxybenzoyl-phenyl

## (C) Of the ester type, i. e.,

Derived from hydroxy-esters by the removal of the hydroxyl group, as for example, by the removal of the hydroxyl group from the following esters:

(1) Esters of hydroxy acids, e. g.,  
Esters formed by substitution of any of the "R" groups listed above for one or more of the acid hydrogen atoms of the following acids:  
Lactic acid  
Hydroacrylic acid  
Citric acid  
Tartaric acid  
Ricinoleic acid  
Hydroxy-stearic acid  
Hydroxy-chlorstearic acid  
Cyclohexanol carboxylic acids  
Hydroxybenzoic acids  
Salicylic acid  
Hydroxy-phthalic acids  
Hydroxy phenyl-benzoic acids  
Naphthol carboxylic acids

(2) Esters of polyhydroxy alcohols and phenols in which at least one hydroxyl group remains unsubstituted, for example, esters formed by esterifying the following so that at least one hydroxyl group remains in the resulting ester:

Ethylene glycol  
Diethylene glycol  
Propylene glycols  
Butylene glycols  
Poly-hydroxy benzenes  
Dihydroxy-benzenes  
Resorcinol  
Catechol  
Hydroquinone  
Tri-hydroxybenzenes  
Pyrogallol

## III. Sulphur-containing radicles, e. g.,

Any of the examples of oxygen-containing radicles in which at least one oxygen atom has been replaced with sulphur.

Specific examples of sulphur-containing radicles are:

(A) Of the thio-ethyl type  
Thio-phenoxo-phenyl (C<sub>6</sub>H<sub>5</sub>-S-C<sub>6</sub>H<sub>5</sub>-)  
Thio-phenoxo-ethyl (C<sub>6</sub>H<sub>5</sub>-S-C<sub>2</sub>H<sub>5</sub>-)  
Thio-lauroxy-phenyl (C<sub>6</sub>H<sub>5</sub>-S-C<sub>17</sub>H<sub>35</sub>-)  
Thio-t-amyl-phenoxo-phenyl (C<sub>6</sub>H<sub>5</sub>-S-C<sub>6</sub>H<sub>5</sub>-C<sub>4</sub>H<sub>9</sub>-)  
Thio-t-amyl-phenoxo-t-amyl-phenyl



Table II—Continued



(B) Of the thio-ketone type



(C) Of the thio-ester type, e. g., derived from hydroxy-esters of thio-carboxylic acids. Examples of such radicles are:



Where R is methyl, ethyl, butyl, amyl, lauryl, stearyl, naphthyl, etc.

(D) Radicles derived from hydroxy-organic polysulphides by removal of the hydroxy group, e. g.,



where R is hydrogen or an alkyl or cyclo-alkyl group



where R is an alkyl or cyclo-alkyl group and R' is an alkylene group.

The addition agents of this invention may also be characterized by the method of preparation. These addition agents are the phosphorus-containing products reaction products of (a) a trivalent phosphorus-and-halogen-containing reagent with (b) an organic hydroxy or mercapto compound, at least one of which reactants contains a cyclo-aliphatic radicle. The product is further characterized by the fact that it contains phosphorus in trivalent form, and contains a cyclo-aliphatic radicle.

The reactant (a) will preferably have the general formula:



where Y is a halogen, and A' and B' are either the same or different halogens, or the same or different radicles selected from the class consisting of those having the formulas  $XR$  and  $R$  where X is oxygen or sulphur and R is an organic radicle or hydrogen.

The reactant (b) will have the formula  $R'XH$  where R' is an organic radicle and X is either oxygen or sulphur.

The pair of reactants (a) and (b) selected are such that at least one of them contains a cyclo-aliphatic radicle; i. e., at least one of the radicles, 75

R and R' is a cyclo-aliphatic radicle. Preferably the reactant (b) is one in which R' is cyclo-aliphatic.

Examples of the reactant (a) are:



Compounds having the formulas  $ROPCl_2$ ,  $(RO)_2PCl$ ,  $RSPCl_2$ ,  $(RS)_2PCl$ ,  $RPCl_2$  and  $RaPCl$  where R is an organic radicle selected from the list under Table II.

Specific examples of these compounds are those in which R is:



Certain compounds of the class having the formulas  $ROPCl_2$  and  $(RO)_2PCl$  may be prepared by adding an organic hydroxy compound slowly to phosphorous trichloride in such proportions that the molecular ratio of organic hydroxy compound to  $PCl_3$  is two or less. Examples of such reagents are those prepared by adding slowly to one mole of phosphorus trichloride one or two moles of a hydroxy-ester, such as, for example:



Examples of the reactant (b) are those having the formula  $R'OH$  and  $R'SH$ , where R' is any cyclo-aliphatic radicle selected from the list under Table II. Specific examples of such compounds are:



When the reactant (a) with which (b) is to be reacted is one which contains a cyclo-aliphatic radicle, the reactant (b) may be selected from any of those having the formulas  $R'OH$  and  $R'SH$  in which  $R'$  is any organic radicle; for example  $R'$  may be any radicle selected from those listed under Table II. Specific examples of reactant (b) to be used in this way are:

n-Octyl alcohol  
Capryl alcohol  
Lauryl alcohol  
Benzyl alcohol  
Phenol alcohol  
Cresols alcohol  
Amyl phenols  
Methyl lactate  
Methyl salicylate

From the foregoing it will be observed that a very large number of specific addition agents are contemplated for use by this invention. This large number of specific materials may be conveniently divided into a number of groups. The criteria which determine the allocation of a specific material to a particular group may generally be considerations such as (a) the precise nature of the material, (b) the mode of its manufacture, and (c) its particular utility.

I shall therefore in the further identification of the numerous specific examples contemplated for use refer to them by groups.

#### Group 1

The addition agents of this group may be subgenerically defined as the oil-soluble phosphorus bearing products resulting from the reaction of a trivalent phosphorus-and-halogen-containing compound with a material of the class consisting of cyclohexanol, homologs of cyclohexanol, mixtures of cyclohexanol and its homologs, and mixtures of homologs of cyclohexanol.

#### Group 2

The addition agents of this group may be subgenerically defined as those which contain sulphur; for example the oil-soluble phosphorus-and-sulphur-containing products resulting from the reaction of a trivalent phosphorus-and-halogen containing compound with a material of the class consisting of cyclohexanol, homologs of cyclohexanol, mixtures of cyclohexanol and its homologs, and mixtures of homologs of cyclohexanol.

#### Group 3

The addition agents of this group may be subgenerically defined as those which contain a halogen; for example the phosphorus-and-chlorine-containing products resulting from the reaction of a trivalent phosphorus-and-halogen containing reagent with chlor-phenyl cyclohexanol.

#### Group 4

The addition agents of this group may be subgenerically defined as those which contain a metal; for example the oil-soluble salts derived from the phosphorus-containing products of the reaction of trivalent phosphorus-and-halogen-containing reagents with cetyl-cyclohexanol.

A particular material or class of materials found especially suitable for use in accordance with this invention and falling within Group 1 as previously identified is the reaction product of  $PCl_3$  and cyclohexanol, this material being for

convenience in identification hereinafter referred to as P. C. Y. In the preparation of this material the commercial grade of cyclohexanol may be employed since it contains in addition to cyclohexanol minor amounts of certain of the homologs such as methyl cyclohexanol.

The relative proportions of this commercial grade of cyclohexanol and  $PCl_3$  used in the preparation of P. C. Y. are given in the following table, as well as the properties of the end product:

|    |                                            |                            |                     |
|----|--------------------------------------------|----------------------------|---------------------|
| 15 | Cyclohexanol                               | parts by weight            | 1215                |
|    | $PCl_3$                                    | do                         | 2655                |
|    | Weight of product                          | do                         | 2545                |
| 15 | Weight of material removed by distillation | do                         | 514                 |
|    | Percent yield based on $PCl_3$             | per cent                   | 84                  |
|    | Percent yield based on $C_6H_{11}OH$       | do                         | 88                  |
| 20 | Boiling point                              | °C                         | 150-165             |
|    | Melting point                              | Liquid at room temperature |                     |
|    | Sp. gr. at 24° C                           |                            | 1.06                |
|    | Color                                      |                            | Light yellow        |
|    | Phosphorus                                 | per cent                   | 11.6                |
| 25 | Chlorine                                   | do                         | 5.6                 |
|    | Acid number                                |                            | 166                 |
|    | Solubility:                                |                            |                     |
|    | $H_2O$                                     |                            | Insoluble           |
|    | Ethyl alcohol                              |                            | Completely miscible |
| 30 | Mineral oil                                |                            | At least 5%         |

The cyclohexanol is placed in a reaction vessel equipped with an agitator and reflux condenser. The vessel and agitator are preferably of glass or enamel. The  $PCl_3$  is added slowly and the temperature of the reactants maintained between 50° C. and 60° C. during the addition of the  $PCl_3$ . The mixture is stirred continuously during the addition of the  $PCl_3$ . The temperature of the reactants may be controlled by the rate of the addition of the  $PCl_3$ . After all of the  $PCl_3$  has been added in the manner above described the reacting materials are heated in a water bath to 100° C. and then by use of such water bath maintained at a temperature of 100° C. for three hours. The reactants are mechanically agitated throughout the periods of addition of  $PCl_3$ ; elevation to 100° C.; and the three hour period while maintained at 100° C.

After being maintained at 100° C. for three hours the reaction material is distilled at an absolute pressure of eight inches of mercury and all materials boiling below 70° C. are discarded. A sharp break in the vapor temperature will be noted indicating completion of the distillation of the low boiling fraction and the fact that the residue is the end product suitable for use. The material which is distilled over is probably largely minor amounts of unreacted  $PCl_3$  and cyclohexanol. If desired the end product may be water washed since such water washing step will be found to remove a certain amount of chlorine which would otherwise remain. The properties of the composition given in the foregoing table are those for material which has been water washed.

We believe that the principal products of the reaction of  $PCl_3$  with a compound of the class consisting of cyclohexanol and homologs of cyclohexanol are esters of phosphorous acid (such as  $(RO)_3P$ ,  $(RO)_2POH$  and  $ROP(OH)_2$ , where R is the cyclohexyl radicle or a homolog of it), and that halogen-bearing derivatives of such esters may also be formed, as well as other halogen-bearing derivatives of  $ROH$ , for example  $RCl$ . It appears that the phosphorus-bearing constitu-

ents of the reaction product are responsible for the stabilizing effect when the product is used in accordance with our invention. However, for most purposes, the other constituents are not deleterious, and for some purposes may even be advantageously included. The phosphorus-bearing constituents are in general much less volatile than the other constituents; the latter may therefore be easily removed, if desired, by distillation at atmospheric or sub-atmospheric pressure.

The following table gives the results obtained by the addition of minor amounts of P. C. Y. prepared as above indicated to several different representative commercial oils and oils treated with other addition agents.

adjusted to maintain a value of 12.7 to 1. In the first test, a S. A. E. 20 motor oil having a viscosity index of about 105 was employed as the lubricant and in a second test, the same oil to which .03% of P. C. Y. was added was employed as a lubricant. The engine was fitted with new pistons and rings before the start of each test and after completion of the first test, the engine was taken down, thoroughly cleaned and fitted with a new piston and rings.

At the conclusion of the first test, nearly the entire skirt of the piston was very black, while at the end of the second test only 60% of the skirt showed only very light deposits of light brown material. The inside of the piston skirt at the end of the first test showed a light shellac-like

| Example No.                    | Composition                    |                             |                    |                   |                    | Oxidation tests     |       |                        |                |                               |                    |                     |                   | Corro-<br>sion test,<br>Lead-<br>Bronze |       |
|--------------------------------|--------------------------------|-----------------------------|--------------------|-------------------|--------------------|---------------------|-------|------------------------|----------------|-------------------------------|--------------------|---------------------|-------------------|-----------------------------------------|-------|
|                                | Hexachlor<br>Diphenyl<br>Oxide | Ortho<br>Dichlor<br>Benzene | Methyl<br>Stearate | Butyl<br>Stearate | Per<br>cent<br>PCY | Conradson<br>Carbon |       | Vis. in SUS at 210° F. |                |                               | Naphtha Insolubles |                     |                   |                                         |       |
|                                |                                |                             |                    |                   |                    | Orig.               | Final | Orig.                  | At 48<br>Hours | Per cent<br>Visc.<br>Increase | Hrs. for<br>10 mg. | Hrs. for<br>100 mg. | Weight<br>48 hrs. |                                         |       |
| MID-CONTINENT SAE 30 MOTOR OIL |                                |                             |                    |                   |                    |                     |       |                        |                |                               |                    |                     |                   |                                         |       |
| 1 (untreated)                  |                                |                             |                    |                   | .03                | .32                 | 1.67  | 63.1                   | 74.4           | 17.9                          | 13.5               | 44                  | 121               | -.18                                    |       |
| 2                              |                                |                             |                    |                   | .06                | .37                 | 1.16  | 62.9                   | 68.8           | 9.4                           | 26.5               | (b)                 | 41                | -.16                                    |       |
| 3                              |                                |                             |                    |                   | .06                | .27                 | 1.30  | 63.5                   | 67.9           | 6.9                           | 24.0               | (b)                 | 94                | -.15                                    |       |
| 4                              | .30                            | .30                         |                    |                   | .06                | .68                 | 1.82  | 63.6                   | 73.1           | 16.0                          | 17                 | 46                  | 111               | -.51                                    |       |
| 5                              | .30                            | .30                         |                    |                   | .06                | .45                 | 1.27  | 62.7                   | 67.9           | 8.3                           | 22                 | (b)                 | 79                | -.22                                    |       |
| 6                              | .50                            | .50                         | .25                | .25               | .03                | .41                 | 2.05  | 61.6                   | 72.2           | 17.2                          | 13                 | 45                  | 118               | -.02                                    |       |
| 7                              | .50                            | .50                         | .25                | .25               | .03                | .40                 | 1.30  | 62.1                   | 69.0           | 11.1                          | 28.5               | (b)                 | 76                | -.23                                    |       |
| PENNSYLVANIA SAE 40 MOTOR OIL  |                                |                             |                    |                   |                    |                     |       |                        |                |                               |                    |                     |                   |                                         |       |
| 8 (untreated)                  |                                |                             |                    |                   |                    | 1.25                | 3.52  | 82.7                   | 104.0          | 29.3                          | (a)                | (b)                 | 5                 | -.08                                    |       |
| 9                              |                                |                             |                    |                   |                    | .03                 | 1.26  | 2.20                   | 84.3           | 95.3                          | 13.1               | (a)                 | (b)               | 3                                       | -.31  |
| 10                             |                                |                             |                    |                   |                    | .06                 | 1.46  | 2.31                   | 81.8           | 95.1                          | 16.3               | (a)                 | (b)               | 2                                       | -.25  |
| 11                             | .30                            | .30                         |                    |                   |                    | .06                 | 1.67  | 3.54                   | 82.3           | 104.0                         | 26.5               | (a)                 | (b)               | 3                                       | -.38  |
| 12                             | .30                            | .30                         |                    |                   |                    | .06                 | 1.66  | 2.61                   | 82.1           | 95.2                          | 16.0               | (a)                 | (b)               | 4                                       | -.16  |
| 13                             | .50                            | .50                         | .25                | .25               |                    | .03                 | 1.19  | 2.80                   | 79.6           | 98.9                          | 24.2               | (a)                 | (b)               | 6                                       | -.35  |
| 14                             | .50                            | .50                         | .25                | .25               |                    | .03                 | 1.63  | 2.41                   | 81.7           | 93.6                          | 14.6               | (a)                 | (b)               | 2                                       | -.18  |
| PENNSYLVANIA SAE 10 MOTOR OIL  |                                |                             |                    |                   |                    |                     |       |                        |                |                               |                    |                     |                   |                                         |       |
| 15 (untreated)                 |                                |                             |                    |                   |                    | .23                 | .94   | 46.3                   | 49.6           | 7.0                           | 26.0               | (b)                 | 54                | -.75                                    |       |
| 16                             |                                |                             |                    |                   |                    | .03                 | .16   | .52                    | 46.1           | 47.7                          | 3.5                | 43                  | (b)               | 12                                      | -.15  |
| 17                             |                                |                             |                    |                   |                    | .06                 | .17   | .43                    | 46.2           | 48.3                          | 4.6                | 39                  | (b)               | 11                                      | -.15  |
| 18                             | .30                            | .30                         |                    |                   |                    | .06                 | .15   | 1.40                   | 46.3           | 50.6                          | 9.3                | 22                  | (b)               | 65                                      | -.140 |
| 19                             | .30                            | .30                         |                    |                   |                    | .06                 | .22   | .58                    | 46.1           | 47.5                          | 3.0                | 34.5                | (b)               | 12                                      | -.22  |
| 20                             | .50                            | .50                         | .25                | .25               |                    | .03                 | .21   | 1.19                   | 46.5           | 50.0                          | 7.5                | 23.0                | (b)               | 85                                      | -.140 |
| 21                             | .50                            | .50                         | .25                | .25               |                    | .03                 | .18   | .55                    | 46.1           | 47.5                          | 3.0                | 41.0                | (b)               | 14                                      | -.23  |

(a) did not produce 10 mg. in 48 hours. (b) did not produce 100 mg. in 48 hrs.

The determinations which appear in the foregoing table, such as, for example, Conradson carbon, viscosity determinations, and naphtha insoluble, were determined on samples prepared by an oxidation test procedure which is in every respect similar to that prescribed by the Standard of Indiana oxidation test, excepting that a piece of iron wire is submerged in the oil during the test. The data given in the column headed "corrosion" has been determined in accordance with the standard Shell corrosion test using lead bronze as the metal.

The effectiveness of P. C. Y. in improving the properties of a lubricating composition for use in internal combustion engines with particular regard to the stability of the lubricant during use has been demonstrated by tests conducted on a liquid-cooled single cylinder 4-cycle gasoline engine rated at 2½ H. P. at 1800 R. P. M. This engine was run at 1600 R. P. M. under a load of 2 H. P. for a period of 100 hours for each test. The cooling fluid temperature was maintained at 250° F. and the temperature of the lubricant in the crankcase at 225° F. The air-fuel ratio was

deposit with a dark brown deposit on the vertical ribs while the inside of the piston skirt at the end of the second test showed no discoloration.

In general, the materials of this invention will not be found incompatible with commonly employed anti-oxidants such as are used in gasolines and the like.

In general, we have found that the materials of the present invention do not detrimentally affect the extreme pressure characteristics of a mineral lubricating oil, for example, which characteristics are the result of the presence therein of the extreme pressure addition agents above-named. Moreover, where the materials of the present invention have been tested in lubricating compositions which also contain certain other addition agents, the extreme pressure characteristics of the resultant composition has been somewhat improved and such improvement has been traceable to the presence therein of the compounds of the present invention.

Throughout the foregoing specification and in the appended claims, reference is made to "oil-soluble" and by such term, as used herein, it is

intended to indicate the ability of the thus defined material to form not only true solutions with the oil to which the same are added, but also the ability to form therewith any form of substantially permanently homogeneous composition.

As indicated above, my invention also contemplates the production and use of oil-soluble derivatives of the compounds above specifically identified. Such derivatives include the oil-soluble salts and ester-salts which may be produced by substituting a metal or basic radicle for one or more of the alcohol derived radicles of the immediate reaction product of  $\text{PCl}_3$  and the alcohol. This is conveniently accomplished by partly or completely saponifying such reaction product with an alkali (e. g., sodium potassium, ammonium or substituted ammonium hydroxide) in aqueous solution. Similar salts and ester-salts of metals other than the alkyl metals may be formed directly by reacting said immediate reaction product with the metallic base, or more readily by double decomposition of the alkyl salt (or ester-salt) with a salt of the other metal.

The reaction product of  $\text{PCl}_3$  prepared in the manner above described is for certain uses preferable over pure tricyclohexyl phosphite.

It will be found that the products resulting from the reaction of  $\text{PCl}_3$  with homologs of cyclohexanol and particularly mixtures of such homologs and mixtures of such homologs with cyclohexanol will produce materials which are quite preferable over the remaining compounds of the class previously identified. The halogen-containing reaction products, whether such halogen is present as a result of the  $\text{PCl}_3$  reaction or introduced by direct halogenation, will be found to give decidedly improved results. In view of the character of the reaction products of  $\text{PCl}_3$  with the homologs of cyclohexanol as well as the halogen-bearing derivatives above referred to, they may be employed in concentrations considerably greater than those previously specified for the entire class of compounds which may be employed as addition agents to lubricating compositions.

Throughout the foregoing description where "halogens" have been referred to, it is to be understood that the chlorinated species are very much preferred although the brominated and fluorinated species will also be found to have utility for particular uses.

The materials to which this invention relates have been found to be particularly effective in preventing corrosion when added to lubricants and fuels employed in internal combustion engines. They have been found to be particularly effective as corrosion inhibitors when added to engine fuels such as gasoline which normally tend to show corrosive effects in which the fuel is burned.

Attention is directed to the fact that I am filing even date herewith an application Serial No. 424,824, which relates to these same materials and it is intended that this application include all of the disclosure of such other application filed even date herewith insofar as the present case does not include the disclosures of such other case. This application is a continuation-in-part of my co-pending application Serial No. 265,051, filed March 30, 1939, now Patent No. 2,290,872.

Other modes of applying the principle of my invention may be employed instead of the one explained, change being made as regards the composition and method herein disclosed, provided

the ingredients or steps stated by any of the following claims or the equivalent of such stated ingredients or steps be employed.

I therefore particularly point out and distinctly claim as my invention:

1. A lubricating composition comprising principally a liquid hydrocarbon of the character which is normally subject to deterioration especially at high temperatures and when in contact with metals, and which has been stabilized against such deterioration by the inclusion therein of a minor amount, sufficient to effect such stabilization, of a mixture phosphorus-containing compounds, which mixture consists of at least a part of the reaction product of (a) a trivalent phosphorus-and-halogen-containing reagent containing an organic radicle selected from the class consisting of aromatic and aliphatic radicles with (b) a cycloaliphatic compound containing the  $-\text{X}-\text{H}$  group where  $\text{X}$  is an element selected from the class consisting of oxygen and sulphur, said reaction product prepared by mixing the reactants and exposing the mixture to reaction conditions which produce the primary reaction product without any substantial decomposition of such primary reaction product.

2. A lubricating composition comprising principally a liquid hydrocarbon of the character which is normally subject to deterioration especially at high temperatures and when in contact with metals, and which has been stabilized against such deterioration by the inclusion therein of a minor amount, sufficient to effect such stabilization, of an organic compound having the following structure:



wherein  $\text{X}$  is an element of the class consisting of oxygen and sulphur;  $\text{P}$  is phosphorus;  $\text{A}$  is a cyclo-aliphatic radicle;  $\text{B}$  is a radicle selected from the class consisting of hydrogen, a metal and organic radicles, and  $\text{C}$  is selected from the class consisting of aromatic and aliphatic radicles.

3. A lubricating composition in accordance with claim 2 in which the cycloaliphatic radicle contains the cyclohexyl nucleus.

4. A lubricating composition in accordance with claim 1 in which (a) is a reagent having the structure  $(\text{RX})_x\text{PCl}_y$  in which  $y$  is a whole number less than three and  $x$  and  $y$  equals three,  $\text{R}$  is an organic radicle selected from the class consisting of aromatic and aliphatic radicles and  $\text{X}$  is selected from the class consisting of oxygen and sulphur.

5. A lubricating composition in accordance with claim 1 in which (b) is a cycloaliphatic alcohol.

6. A lubricating composition in accordance with claim 1 in which (b) is an alcohol containing the cyclohexyl nucleus.

7. A lubricating composition in accordance with claim 1 in which (b) is a substituted cyclohexyl alcohol.

8. A lubricating composition in accordance with claim 1 in which (b) is a cycloaliphatic ester.

9. A lubricating composition in accordance with claim 1 in which (b) is a cycloaliphatic mercaptan.

10. A lubricating composition in accordance with claim 1 in which (b) is a mercaptan containing a cyclohexyl nucleus.

11. A lubricating composition in accordance with claim 1 in which (a) is the reaction product

13

of trimethyl citrate with phosphorus trichloride and (b) is cyclohexanol.

12. A lubricating composition in accordance with claim 1 in which (a) is the reaction product of methyl lactate with phosphorus trichloride and (b) is cyclohexanol.

13. A lubricating composition comprising principally a liquid hydrocarbon of the character which is normally subject to deterioration especially at high temperatures and when in contact with metals, and which has been stabilized against such deterioration by the inclusion therein of a minor amount, sufficient to effect such stabilization, of a material of the class consisting of (1) a mixture of phosphorus-containing compounds, which mixture consists of at least a part of the reaction product of (a) a trivalent phosphorus-and-halogen-containing reagent containing an organic radicle selected from the class consisting of aromatic and aliphatic radicles with (b) a compound of the class consisting of cycloaliphatic hydroxy and cycloaliphatic mercapto compounds said reaction product prepared by mixing the reactants and exposing the mixture to reaction

14

conditions which produce the primary reaction product without any substantial decomposition of such primary reaction product, (2) salts derived from (1), and (3), halogen-bearing derivatives of (1) and (2).

5 DELTON R. FREY.

## REFERENCES CITED

The following references are of record in the 10 file of this patent:

## UNITED STATES PATENTS

| Number       | Name           | Date          |
|--------------|----------------|---------------|
| 2,178,610    | Salzberg       | Nov. 7, 1939  |
| 2,290,872    | Frey           | July 28, 1942 |
| 2,285,853    | Downing        | June 9, 1942  |
| 15 2,191,996 | Shoemaker      | Feb. 27, 1940 |
| 2,285,854    | Downing        | June 9, 1942  |
| 2,263,618    | Downing et al. | Nov. 25, 1941 |
| 20 2,199,944 | Peski          | May 7, 1940   |
| 2,261,047    | Asseff         | Oct. 28, 1941 |
| 2,223,793    | Perry          | Dec. 3, 1940  |
| 2,226,543    | Ashburn        | Dec. 31, 1940 |
| 2,220,851    | Schreiber      | Nov. 5, 1940  |